

## UNITED STATES PATENT OFFICE.

STANLEY ERNEST DAWSON, OF DAVENPORT, STOCKPORT, ENGLAND, ASSIGNOR, BY MESNE ASSIGNMENTS, TO FERRANTI METER AND TRANSFORMER MANUFACTURING COMPANY, LIMITED, OF TORONTO, CANADA.

## MACHINABLE NONMAGNETIC HIGH-RESISTANCE CAST-IRON ALLOY.

No Drawing. Application filed November 25, 1921. Serial No. 517,777.

To all whom it may concern:

Be it known that I, STANLEY ERNEST DAWSON, a subject of the King of Great Britain and Ireland, and residing at The Cottage, 5 Frewland Avenue, Davenport, Stockport, in the county of Chester, England, have invented a certain new and useful Machinable Nonmagnetic High-Resistance Cast-Iron Alloy, of which the following is a specification.

This invention relates to an alloy having iron as its principal constituent, which is non-magnetic or nearly so, and has a high specific electrical resistance, and which resembles cast iron as regards its treatment in the foundry and by cutting tools either machine or hand operated.

Articles made of such alloy when subject to the influence of an alternating magnetic field have only small currents induced in them. They may, therefore, be advantageously used instead of similar articles made of brass for use in electrical apparatus, as thereby eddy current losses are greatly reduced.

It is well known that an alloy having iron as its principal constituent and with a certain proportion of manganese is practically non-magnetic, but articles cast from such alloys are too hard to be machined by the usual workshop cutting tools and can only be operated on by grinding.

The invention consists in a non-magnetic or nearly non-magnetic alloy resembling cast iron as regards its treatment in the foundry and workshop, having a higher specific electrical resistance than cast iron, and having as its essential constituents iron, manganese or its equivalent and another metal or metals, for example nickel.

The invention also consists in articles made from such alloy, for use in electrical apparatus.

A suitable alloy according to my invention contains iron, manganese and nickel, in the proportions 85, 5 and 10 respectively. It also contains carbon, silicon and other ingredients of minor or non-essential character as usually found in ordinary cast iron.

The alloys made according to my invention are of the nature of cast iron as regards the physical properties which affect the foundry and machine shop operation. Manganese is present in such proportion as to

give the desired non-magnetic quality, and 55 nickel in such proportion as to counteract the hardening effect of the manganese and render the alloy susceptible to treatment by cutting tools as is cast iron. The presence of nickel reduces the amount of manganese 60 otherwise necessary to make the alloy non-magnetic. An alloy consisting mainly of iron and manganese requires a much greater proportion of manganese to make it non-magnetic than do alloys made according to 65 my invention. In fact, the known iron-manganese alloys with a high percentage of manganese do not possess anything like the same degree of non-magnetic quality as does an alloy made according to my invention 70 with the proportions stated above.

An alloy of the proportions stated above is practically non-magnetic, has a specific electrical resistance nearly twice that of ordinary cast iron, twenty times that of 75 brass, or one hundred times that of pure copper. Its tensile strength is about 14.5 tons per square inch, and its ductility is superior to that of cast iron. It has a very close grain, and can be machined as easily 80 as soft cast iron. The softness can be increased by increasing the nickel content.

For articles in which the highest possible degree of non-magnetic quality is not essential a less costly alloy can be used. As an 85 example, the following relative proportions can be used:—iron 90, manganese 5, nickel 5.

One method of producing an alloy according to my invention consists in melting the metals other than cast iron (that is, manganese and nickel) in a crucible and adding such molten metal to ordinary molten cast iron as it flows into the ladle from the spout of the cupola in which it has been melted.

Having now described my invention, what I claim as new and desire to secure by Letters Patent is:—

1. A practically non-magnetic machinable cast iron-like alloy containing manganese in amount to render the alloy substantially non-magnetic, the balance of the alloy being principally of cast iron, and a metal 100 to render the alloy machinable.

2. A practically non-magnetic cast iron-like alloy containing manganese in amount to render the alloy substantially non-magnetic, the balance of the alloy being prin- 105

- cipally of cast iron and nickel to render the alloy machinable.
3. An article for use in electrical apparatus made of non-magnetic machinable cast iron-like alloy containing manganese in amount to render the alloy substantially non-magnetic, the balance of the alloy being principally of cast iron and a metal to render the alloy machinable.
- 10 4. A practically non-magnetic machinable cast iron alloy including from 5 to 14% of nickel, between 3 and 7% of manganese and at least 80% of grey cast iron.
5. A practically non-magnetic machinable cast iron alloy as claimed in claim 4, in which the cast iron contains at least 2.5% of carbon and at least 1.5% of silicon.
6. A practically non-magnetic machinable cast iron alloy including 85% of iron, at least 1.5% of silicon, 5% of manganese and 10% of nickel.
7. Articles for use in electrical apparatus made from an alloy as claimed in claim 4.

In testimony whereof I have signed my name to this specification.

STANLEY ERNEST DAWSON.